

## UNITED STATES PATENT OFFICE

2,576,419

## CLEANING COMPOSITION

John Henry Sechrist and Wilbur Herbert Petering;  
 Detroit, Mich., assignors to Detrex Corporation,  
 Detroit, Mich., a corporation of Michigan

No Drawing. Application June 4, 1947;  
 Serial No. 752,568

1. Claim. (Cl. 252—118)

**1.** This invention relates to improved cleaning compositions and particularly to new metal cleaning and dry cleaning compositions containing a chlorinated hydrocarbon solvent, a detergent and water, the finished composition being in "sub-emulsion" form as hereinafter defined and described.

In the art of cleaning metals by the use of a solvent and also in the art relating to the dry-cleaning of clothes with a solvent it has been thought for many years that it was necessary to avoid the presence of water. In the case of metal cleaning the presence of water in its usual form in such solvents leads to negative cleaning and to undesirable decomposition reactions, particularly where the solvent is a chlorinated hydrocarbon. There is also a danger of corrosion of the metal in using such compositions in the presence of water. In the case of liquid dry-cleaning compositions, the presence of water in its usual form produces undesirable shrinkage of the material being cleaned. Prior attempts to incorporate water into cleaning compositions containing such solvents have therefore been directed to the production of various soaps containing chlorinated hydrocarbon compounds and also to more or less turbid emulsions containing soap and a solvent such as a chlorinated hydrocarbon. For a number of reasons compositions of the soap type and of the turbid emulsion type have not been satisfactory and we therefore do not intend to include such compositions within the scope of the present invention which is directed to sub-emulsion cleaning compositions and their use.

We have found that the difficulties of the prior art are avoided and a greatly improved cleaning operation is obtained both on metals and on clothes and the like when water and a detergent are incorporated in a chlorinated hydrocarbon composition in what we have in this specification termed as a "sub-emulsion" characterized by a clear liquid appearance in the final form and lacking any visible appearance of turbidity or of particle suspension. The sub-emulsion of the present invention is obtained by incorporating water into a chlorinated hydrocarbon solvent with the aid of a suitable coupler. This constitutes the basic sub-emulsion cleaning composition of the present invention. It may be necessary to add a detergent if the coupler is not a detergent and where this is done a detergent soluble in the basic sub-emulsion is selected or a suitable coupler is used for coupling the detergent into the sub-emulsion, thereby pre-

10  
 15  
 20  
 25  
 30  
 35  
 40  
 45  
 50  
 55

serving the sub-emulsion form. However, it is possible to select a solvent-water coupler having detergent properties and where this is done the addition of a second detergent is not necessary. The resulting cleaning composition is a perfectly clear, easily flowing liquid and appears to derive its superior cleaning qualities, in part at least, from the nature of the interface between the chlorinated hydrocarbon and the water and this interface is one of the elements of our sub-emulsion. As specific examples we have found the following to be of particular value.

*Example 1*

|    |                               |       |     |
|----|-------------------------------|-------|-----|
| 15 | Trichlorethylene (stabilized) | cc    | 100 |
|    | Triethanolamine oleate        | grams | 2   |
|    | Monoethanolamine oleate       | do    | 6   |
|    | Sodium oleate                 | gram  | 1   |
|    | Water                         | cc    | 11  |

The above ingredients are mixed by first dissolving the triethanolamine oleate and the monoethanolamine oleate in the trichlorethylene. The sodium oleate is then dissolved in the water and this solution is mixed with vigorous agitation with the previously prepared trichlorethylene solution until a sub-emulsion form is reached. The formation of the sub-emulsion may be accelerated by the use of heat. The final liquid sub-emulsion is clear, has a yellowish-orange color, has a specific gravity of 1.38 and foams on agitation. Such foaming decreases as the composition is used and is not objectionable. For most metals the final sub-emulsion is non-corrosive when properly used as a cleaning composition.

*Example 2*

|    |                               |     |     |
|----|-------------------------------|-----|-----|
| 40 | Trichlorethylene (stabilized) | gal | 45  |
|    | Oleic acid                    | lb  | 27  |
|    | Triethanolamine               | lb  | 2.6 |
|    | Monoethanolamine              | lb  | 4.0 |
|    | Sodium hydroxide              | oz  | 7.9 |
|    | Water                         | gal | 5   |

The triethanolamine and the monoethanolamine are added to the oleic acid with vigorous stirring. The sodium hydroxide is then dissolved in the water and added to the above mixture with vigorous stirring until a white homogeneous paste is obtained. This paste is then added to the trichlorethylene and stirred until a clear sub-emulsion liquid is obtained. The addition of a small amount of heat reduces the stirring time required for obtaining the clear liquid characteristic of the sub-emulsion form.

In the above examples the triethanolamine oleate serves primarily as a coupler for the oleic acid soap and the trichlorethylene. The monoethanolamine oleate serves primarily as a coupler for the water and the trichlorethylene, but it also has valuable cleaning characteristics. In this connection we have found that monoethanolamine oleate is far superior to triethanolamine oleate in producing and maintaining the sub-emulsion of this invention. This we believe is due in part to the fact that this compound has a polar group at one end of its molecular structure and a non-polar group at the other end. Its detergent properties are such that it is possible to omit the oleic acid, the sodium hydroxide and the triethanolamine from the above composition leaving the monoethanolamine oleate to act as a coupler and a detergent. The composition so attained comprises 45 gallons trichlorethylene, 5 gallons water, and 22 pounds monoethanolamine oleate, 4 pounds monoethanolamine combining with approximately 18 pounds of oleic acid to produce 22 pounds of monoethanolamine oleate. Where this is done the cleaning composition consists of a chlorinated hydrocarbon solvent, water and a coupler having detergent properties. The relative amount of water is limited to the amount which can be maintained in the composition in sub-emulsion form, herein defined as optically clear, non-turbid liquid.

We have found that the cleaning efficiency of the above compositions is far superior to that of any of the ingredients separately or to the cleaning efficiency of the same ingredients combined in other physical compositions such as pastes or turbid emulsions where the composition is not in sub-emulsion form. For instance, where soap is added to the usual emulsion there is no outstanding improvement in cleaning whereas soap added to our sub-emulsion in proper amount results in greatly improved cleaning. In the cleaning of clothes and the like the removal of water soluble stains is greatly enhanced and in the metal cleaning field the removal of smut and the like is greatly improved. This latter action probably results from the sub-emulsion interface. In this connection we have found that there is a limiting amount of water which can be used depending on the concentration of soap present. For instance we have found that the maximum amounts of water for the formation of a sub-emulsion where triethanolamine oleate is present in the composition increase with the soap concentration. Where only monoethanolamine oleate is present, significantly larger amounts of water may be incorporated in sub-emulsion form and these amounts also increase as the soap concentration is increased. At all events, it is important that the relative amount of water be limited to that which can be maintained in the composition in sub-emulsion form.

It will be understood that other chlorinated hydrocarbons such as tetrachlorethylene, tetrachlorethane, pentachlorethane and carbon tetrachloride may be used in place of trichlorethylene

and that other well known soaps may be substituted for the sodium oleate. We have also found that sodium abietate and cyclic hydroxy compounds such as cresol and cyclohexanol make satisfactory couplers in the composition of our invention.

It will be noted that the chlorinated hydrocarbon used in the above example, namely trichlorethylene, is designated as "stabilized." Such stabilization is particularly desirable where the finished composition is to be used in vapor degreasing operations for the cleaning of metals and may be accomplished by the addition of small amounts of known stabilizers such as pyridine or triethylamine as described in U. S. Patent Number 2,096,735. Where other chlorinated hydrocarbons are used in producing the sub-emulsions referred to it may be desirable to use other stabilizers as described in the patent referred to above.

The term "sub-emulsion" as used throughout this specification and the appended claim is intended to define a composition containing a chlorinated hydrocarbon to which water has been coupled in an amount which results in a perfectly clear, non-turbid, easily flowing liquid. In some cases such sub-emulsions may be colored but even where colored there is an absence of visible particles or turbidity. In forming the sub-emulsion of the present invention it is first necessary to use a highly efficient coupler for the solvent and the water. If the coupling agent is not a detergent, it is then necessary to include a detergent in the finished sub-emulsion and this detergent must either be soluble in the sub-emulsion or must be coupled into it by means of a suitable coupling agent.

Having thus described our invention, we claim:  
An optically clear, non-turbid, liquid, cleaning composition comprising the following ingredients

40 in substantially the proportions stated:

|                         |       |     |
|-------------------------|-------|-----|
| Trichlorethylene        | cc    | 100 |
| Triethanolamine oleate  | grams | 2   |
| Monoethanolamine oleate | do    | 6   |
| Sodium oleate           | gram  | 1   |
| Water                   | cc    | 11  |

JOHN HENRY SECRIST.  
WILBUR HERBERT PETERING.

#### REFERENCES CITED

The following references are of record in the file of this patent:

#### UNITED STATES PATENTS

| Number    | Name       | Date          |
|-----------|------------|---------------|
| 1,847,437 | Moscowitz  | Mar. 1, 1932  |
| 1,911,289 | Reddish    | May 30, 1933  |
| 2,070,908 | Levine     | Feb. 16, 1937 |
| 2,107,287 | Curran     | Feb. 8, 1938  |
| 2,374,113 | Lowe       | Apr. 17, 1945 |
| 2,383,114 | DeVilliers | Aug. 21, 1945 |

#### OTHER REFERENCES

Emulsions, Booklet of Carbide & Carbon Chem. Corp., N. Y. (1930), pages 21, 22 and 23.